

# UNITED STATES PATENT OFFICE.

CARL HUGGENBERG, OF CHEMNITZ, SAXONY, GERMANY.

## PROCESS OF TREATING SILK FIBER.

SPECIFICATION forming part of Letters Patent No 339,778, dated April 13, 1886.

Application filed September 12, 1885. Serial No. 176,956. (No specimens.)

*To all whom it may concern:*

Be it known that I, CARL HUGGENBERG, of Chemnitz, in the Kingdom of Saxony and Empire of Germany, have invented certain new and useful Improvements in Processes of Treating Silk Fiber Preparatory to Dyeing and Weaving, of which the following is a specification.

This invention relates to a process of treating silk threads preparatory to dyeing and weaving; and it consists in immersing the silk threads in a solution of a suitable tin-salt, and then subjecting the fibers to the action of a solution of tungstate of soda, so as to fix the tin-salts formed thereby in or on the fibers.

In carrying out my invention I prefer to use a solution of tetrachloride of tin, of the strength of 20° Baumé, in which the silk threads are steeped for about an hour. In place of the tetrachloride of tin, the double salts of tetrachloride of tin, or stannate of alkali, containing an equivalent amount of oxide of tin may be employed. The silk threads are, after steeping, withdrawn from the solution and the surplus liquor removed by wringing the hanks, after which they are transferred to a solution of tungstate of soda, of 40° Baumé, in which the hanks also remain for about an hour. The hanks are then wrung so as to remove the surplus liquor, washed, and then again placed in a weaker solution of tetrachloride of tin, or other equivalent tin-salt, of 10° Baumé, and finally placed in a bath of weak muriatic acid formed of three parts of concentrat-

ed muriatic acid and one hundred parts of water, and finally thoroughly washed.

By the formation of tungstate of tin in or on the fibers by the action of the tungstate of soda on the tin-salts referred to the silk fibers are enlarged and adapted to be dyed more evenly, whereby the brilliancy of the color is increased, greater body and durability produced, and the fibers rendered less inflammable.

I am aware that oxides of tin and their hydrates and tungstate salts have been used as a mordant and also as a means for making the fibers non-inflammable, and I do not claim either one of these applications, but confine myself to the fixing of the tin-salt by the tungstate of soda in or on the fibers.

Having thus described my invention, I claim as new and desire to secure by Letters Patent—

The process herein described of treating silk threads, which consists in subjecting the threads to the action of a solution of a suitable tin-salt, and then subjecting them to the action of a solution of tungstate of soda, so as to fix the resulting tin salt in or on the fibers, substantially as set forth.

In testimony that I claim the foregoing as my invention I have signed my name in presence of two subscribing witnesses.

CARL HUGGENBERG.

Witnesses:

RUDOLF KRETZSCHMAR,  
BENNO JOHANES SCHMIDT.